

## UNITED STATES PATENT OFFICE

2,292,213

## YARN CONDITIONING PROCESS AND COMPOSITION THEREFOR

Joseph B. Dickey and James G. McNally, Rochester, N. Y., assignors to Eastman Kodak Company, Rochester, N. Y., a corporation of New Jersey

No Drawing. Application August 15, 1939,  
Serial No. 290,320

3 Claims. (Cl. 252—8.6)

This invention relates to the conditioning of textile yarns and more particularly to the lubrication of filaments and yarns composed of organic derivatives of cellulose such as cellulose acetate, cellulose propionate, cellulose acetate propionate, and cellulose acetate butyrate, to render them more amenable to textile operations such as weaving, knitting and the like.

As is well known in the manufacture of yarns, particularly those composed of or containing cellulose organic derivatives, it is necessary to treat the yarn in order to reduce the tendency toward breakage of the individual filaments or fibers when they are subjected to various mechanical strains and to lubricate the yarn in order to facilitate handling in such operations as spinning, twisting, winding and reeling. It is also necessary to treat yarn to adapt it for use as warp or filling or for the manufacture of various types of knitted fabrics.

This invention has as its principal object to provide an entirely new class of yarn conditioning agents which are particularly adapted for the lubrication of yarns composed of or containing organic derivatives of cellulose. A further object is to provide lubricating formulas which can be readily removed from the yarns by the usual scour baths. Another object is to provide an improved type of yarn which is especially amenable to textile operations including weaving, spinning, knitting and the like. Other objects will appear hereinafter.

These objects are accomplished by the following invention which, in its broader aspects, comprises the discovery that ketones prepared by reacting certain aromatic hydrocarbons such as benzene, naphthalene, diphenyl, triphenyl, anthracene, dibenzofuran, furan, thiophene, acenaphthene, etc., in substituted or unsubstituted form, with naphthenic acid chlorides prepared by reacting a naphthenic acid or mixture of naphthenic acids with an acid chloride-forming reagent such as thionyl chloride, phosphorus pentachloride, phosphorus trichloride, oxalyl chloride, benzoyl chloride, etc., may be used as yarn lubricating agents. In preparing ketones of phenols any suitable modification of the Friedel-Crafts reaction, such as the Frees rearrangement, may be employed, if desired. By the above reference to naphthenic acids we refer to acids such as those described in chapter 48 of the text by Carlton Ellis entitled "The Chemistry of Petroleum Derivatives," first edition (1934), published by the Chemical Catalogue Company, New York, New York.

The ketones thus prepared may be employed as yarn treating agents alone, or in conjunction with other known textile lubricants such as animal, mineral, or vegetable oils and/or various 5 yarn solvent or softening agents such as glycerine, ethylene glycol, polyethylene glycols and their ethers and esters, and similar agents. The oil ingredient of such compounded yarn treating compositions may include sulphonated or un-10 sulphonated oils, phosphated or phosphited blown and unblown vegetable and animal oils and similar materials.

## PREPARATION OF COMPOUNDS

## PHENYL NAPHTHENYL KETONE

Three hundred g. benzene, 67 g. aluminum chloride and 73 g. naphthenic acid chloride are heated with stirring on a steam bath for 10 hours or until no more hydrogen chloride is evolved. 15 When the reaction mixture is cool, it is poured on ice, separated, washed with 5% hydrochloric acid followed by water and distilled. There is obtained an excellent yield of phenyl naphthenyl 20 ketone boiling at 125-300°/1 mm.

## THIENYL NAPHTHENYL KETONE

Seventeen g. thiophene are dissolved in 150 cc. benzene with 40 g. naphthenic acid chloride. 25 There is then added with stirring 26 g. titanium tetrachloride and the reaction is completed by warming. When cool the reaction product is poured onto ice and then worked up as in the preceding paragraph. There is obtained an excellent yield. The resulting thiienyl naphthenyl 30 ketone boils at 130-300°/1 mm.

## PYRROLY NAPHTHENYL KETONE

One equivalent of ethyl magnesium bromide is 35 added to an ether solution of an equivalent amount of pyrrole. Then one equivalent amount of naphthenic acid chloride in dry ether is added slowly with stirring. Stirring is continued at room temperature for 15 hours and then on the water bath for several hours. The reaction mixture is poured onto ice, and hydrolyzed with ammonium chloride. The ether solution is separated from the water, washed with water, and distilled. There is obtained a good yield of pyrroly naphthenyl ketone.

## O- AND P-HYDROXYPHENYLNAPHTHENYL KETONE

Three hundred and seventy-four g. of aluminum chloride and 400 cc. carbon disulfide are placed in a reaction flask and 500 g. phenylnaphthenate are added. The reaction begins and beat

is evolved. When all of the ester has been added, the mixture is heated to refluxing until no more hydrogen chloride is evolved. The carbon bisulfide is removed and the reaction mixture is heated in an oil bath at 140-160° until no more hydrogen chloride is evolved. The mixture is then treated with a mixture of water and hydrochloric acid. After separation, the product is separated and purified by distillation or crystallization. There is obtained a good yield of o- and p-hydroxy-phenylnaphthyl ketone.

#### NAPHTHYL NAPHTHENYL KETONE

Three hundred cc. carbon bisulfide, 67 g. aluminum chloride, 75 g. naphthenic acid chloride and 33 g. naphthalene are allowed to react at room temperature for twenty hours. The reaction product is worked up as in the preceding paragraph. There is obtained a good yield of naphthyl naphthyl ketone.

In a similar manner, triphenyl, anthracene, diphenyl ether, benanthrene, acenaphthene, anisole, carbazole, dibenzofuran, etc., are reacted, and the corresponding compounds obtained.

#### NAPHTHENYL-XYLYL KETONE

1-kg. dry mixed xylene is heated on a steam bath for 24 hours with 400 g. aluminum chloride and 250 g. mixed naphthenic acids. The product is poured onto ice and treated with 5% hydrochloric acid. When hydrolysis is complete the xylene-ketone layer is separated from the water and distilled under reduced pressure. There is obtained an 80-85% yield of naphthyl-xylyl ketone boiling at 200-290°/10 mm.

In accordance with the invention these compounds may be applied directly to the yarn during or after spinning, or may be added to the spinning solution itself. We have found that these compounds have exceptional ability to lubricate textile yarns, particularly those composed of or containing organic derivatives of cellulose such as cellulose acetate, cellulose acetate propionate, cellulose acetate butyrate, and the like. As previously indicated, they may also be employed in connection with the usual yarn lubricating materials, such as mineral oil, and blown and unblown, drying and semi-drying, vegetable and animal oils, fats and waxes.

In the following examples and description, we have set forth several of the preferred embodiments of our invention, but they are included merely for purposes of illustration and not as a limitation thereof.

Our invention will be more readily understood by reference to the following examples in which typical applications of the invention are set forth.

#### Example 1

Phenyl naphthyl ketone is applied to textile materials (silk, wool, cotton, cellulose acetate, viscose, etc.) by means of a bath, wick, roller, spray, etc., to facilitate their knitting, weaving, spinning, and the like. If the yarn is intended primarily for knitting, the amount of conditioning liquid applied may vary from 2 to 25% by weight of the yarn. If the yarn is intended primarily for weaving, the amount of conditioning liquid applied may vary between 1 and 5% by weight of the yarn.

#### Example 2

|                                  |            |
|----------------------------------|------------|
| Olive oil.....                   | Parts 1-99 |
| Xylylnaphthylketone (mixed)..... | 99-1       |

This mixture is applied to textile materials such as silk, wool, viscose, cellulose acetate, etc., as described in Example 1. If the yarn is intended primarily for knitting, the amount of conditioning liquid applied may vary between 2-25% by weight of the yarn, and if for weaving, the amount of liquid applied may vary between 1 and 5% by weight of the yarn. Cellulose acetate filaments or fibers treated as described above are quite soft and pliable and give improved results in various textile operations such as weaving, knitting, etc.

#### Example 3

15 Naphthyl furyl ketone is applied to textile materials such as cellulose acetate, viscose, silk, wool, etc. from a benzene solution as in Example 1. The benzene is removed by passing the materials through a suitable drying cabinet. If the yarn is intended primarily for knitting, the amount of conditioning liquid applied may vary from 2-25% by weight of the yarn. If the yarn is intended for weaving, the amount of conditioning liquid applied may vary between 1 and 5% by weight of the yarn.

20 Other examples of yarn conditioning compositions which may be applied to various types of yarns, particularly those composed of or containing cellulose acetate, cellulose acetate propionate, cellulose acetate butyrate, and similar cellulose organic acid esters in accordance with our invention and which render such yarns especially well adapted for various textile operations such as weaving, knitting, are as follows:

#### Example 4

|                                  | Parts |
|----------------------------------|-------|
| 40 Naphthyl diphenyl ketone..... | 75-99 |
| β-Methoxyethylsuccinate.....     | 25-1  |

#### Example 5

|                               |       |
|-------------------------------|-------|
| Di-naphthyl anthracene.....   | 1-25  |
| 45 Olive oil.....             | 40-45 |
| Tetrahydrofurfurylformal..... | 59-30 |

#### Example 6

|                               |       |
|-------------------------------|-------|
| 50 Naphthyl phenanthrene..... | 1-10  |
| Blown olive oil.....          | 99-90 |

#### Example 7

|                                     |       |
|-------------------------------------|-------|
| 4-hydroxyphenylnaphthyl ketone..... | 1-40  |
| 55 Neat's-foot oil.....             | 99-60 |

#### Example 8

|                                          |       |
|------------------------------------------|-------|
| 2,5-dihydroxy phenylnaphthyl ketone..... | 1-15  |
| Blown neat's-foot oil.....               | 99-85 |

#### Example 9

|                                   |       |
|-----------------------------------|-------|
| p-Cetylphenylnaphthyl ketone..... | 1-50  |
| Mineral oil.....                  | 99-50 |

#### Example 10

|                                      |    |
|--------------------------------------|----|
| Blown sperm oil.....                 | 70 |
| Ethanolamine acetate propionate..... | 25 |
| Naphthyl dibenzoylfuran ketone.....  | 5  |

#### Example 11

|                                              |       |
|----------------------------------------------|-------|
| Sperm oil.....                               | 80-60 |
| Butyl naphthenate.....                       | 5-20  |
| 75 Alkylated naphthalene naphthylketone..... | 5-20  |

*Example 12*

|                                     | Parts |
|-------------------------------------|-------|
| Mineral oil                         | 30    |
| Naphthenyl p-phenoxy phenylketone   | 20    |
| Blown neat's-foot oil               | 40    |
| Oleyl alcohol                       | 5     |
| Tetrahydrofurfuryltetrahydrofuroate | 5     |

*Example 13*

|                                | Parts | Parts |
|--------------------------------|-------|-------|
| Mineral oil                    | 70-50 | 10    |
| Oleic acid                     | 1-25  |       |
| p-Aminophenylnaphthenyl ketone | 29-25 |       |

*Example 14*

|                       | Parts | Parts |
|-----------------------|-------|-------|
| Blown sperm oil       | 25    | 15    |
| Blown olive oil       | 25    |       |
| Blown neat's-foot oil | 25    |       |
| Sodium sulfate        | 2     |       |
| Oleic acid            | 22-13 |       |
| Sulfonated castor oil | 1-10  | 20    |

*Example 15*

|                              | Parts | Parts |
|------------------------------|-------|-------|
| $\beta$ -Methoxyethyladipate | 20    |       |
| Blown neat's-foot oil        | 30    |       |
| Sulfonated olive oil         | 10    |       |
| Mineral oil                  | 10    | 25    |
| Oleic acid                   | 10    |       |
| Phenylnaphthenyl ketone      | 3     |       |
| Ethanol amine                | 7     |       |
| Water                        |       |       |

*Example 16*

A twenty per cent solution of cellulose acetate in acetone in which is incorporated 1-25% by weight of the cellulose acetate of phenyl naphthenyl ketone is extruded through fine orifices into an evaporative atmosphere. The filaments thus produced are wound or twisted and wound. Yarns produced from filaments thus prepared are pliable and suitable for knitting.

Any of the above lubricants may be applied to the yarn by means of a bath, wick, spray, roller, pad or any suitable means. The amount of the lubricant applied may vary between 1% and 25% by weight of the yarn treated.

Although in the above examples, we have referred primarily to yarn treating compositions containing only the lubricating compounds which are the specific subject of this application, together with an oil, other ingredients such as solvents, non-solvents, emulsifying agents, blending agents and the like, may be added within the scope of our invention. Likewise, various dyes or other coloring matter may be included in case it is desired to fugitively or permanently tint or dye the material undergoing treatment.

Although we have found it convenient to illustrate our invention by reference to compositions containing specific percentages of the various ingredients, these percentages may vary widely de-

pending upon the particular purpose for which the composition is intended.

While we have described our invention with particular reference to the treatment of yarns composed of organic derivatives of cellulose such as cellulose acetate, the lubricating formulas described herein are applicable to the lubrication of many other types of cellulose derivative yarns such as those composed of or containing cellulose propionate, cellulose butyrate, cellulose acetate propionate and cellulose acetate butyrate, ethyl, methyl and benzyl celluloses, as well as to the lubrication of silk, wool, cotton, viscose and other natural or synthetic materials.

The term "yarn" as used herein and in the claims is to be understood as including a single filament, a plurality of filaments associated into the form of a thread, either of high or low twist, single or multiple threads associated or twisted together, composite threads composed of a mixture of natural and artificial filaments or a composite thread formed by twisting together individual strands of natural or artificial materials, as well as cut staple fibers produced from natural and/or artificial filaments or threads and spun yarn produced from such staple fibers.

The compositions described herein have been found to possess exceptional ability to lubricate and condition cellulose organic derivatives and other yarns for use in various textile operations such as weaving, knitting, twisting, spinning and the like. Due to the solubility in water of the compositions, they may be readily removed from yarns and fabrics by means of the usual aqueous scour baths. By employing the yarn lubricating agents herein described, one is enabled to obtain highly satisfactory results in the manufacture of yarns and woven fabrics of various kinds.

What we claim is:

1. The process of conditioning textile yarns composed of or containing organic derivatives of cellulose to render them more amenable to textile operations including knitting, weaving, spinning and the like, which comprises applying thereto a yarn lubricating composition containing as its essential lubricating component xylol naphthenyl ketone.
2. Textile yarns composed of or containing organic derivatives of cellulose which are amenable to textile operations including knitting, weaving, spinning and the like, impregnated with a lubricant containing as its essential lubricating component xylol naphthenyl ketone.
3. A textile yarn lubricating composition, the essential lubricating component of which is xylol naphthenyl ketone.

JOSEPH B. DICKEY.  
JAMES G. McNALLY.